# EUROPEAN PATENT SPECIFICATION

(11) **EP 0 383 895 B1**
(45) Date of publication and mention of the grant of the patent: **24.08.1994**
(21) Application number: 89909806.5
(22) Date of filing: 23.08.1989
(51) Int. Cl.: A41D 31/02, A63B 71/08

(54) **METHOD OF MAKING A PROTECTIVE MATERIAL**
HERSTELLUNGSVERFAHREN EINES SCHUTZMATERIALS
PROCEDE DE FABRICATION D'UNE MATIERE DE PROTECTION

(30) Priority: 23.08.1988 GB 8819942
(43) Date of publication of application: 29.08.1990
(73) Proprietor: SPORTS PROTECTION LIMITED, Dunstable, Bedfordshire LU6 3AG (GB)
(72) Inventor: BELL, Keith, Michael 57 Yew Street, Dunstable Bedfordshire LU5 5PA (GB); STANESBY, Gerald, Reginald 256 Dunstable Road, Dunstable Bedforshire LU6 2QG (GB)
(74) Representative: Wain, Christopher Paul
(86) International application number: GB8900977
(87) International publication number: WO9001883

(56) References cited:
- GB-A- 1 556 357
- US-A- 4 441 211
- US-A- 4 507 801

## Description

The present invention relates to a method of making a semi-rigid protective material.

The material is particularly useful for body protection for both humans and animals. Examples are particularly useful for protection against sporting injuries such as in the fields of cricket, football, yachting and motorcycle racing or for protection against attack. For example, the protective material may be formed into shin pads, shoulder pads, arm pads, protective life jackets, body armour, lumbar protectors or back or chest protectors.

It is known to provide protectors of the above types but in general these comprise a very rigid portion. While this may protect against some degrees of injury, there are occasions when the rigid protection snaps or breaks and in fact is likely then to aggravate any injury received.

It is an object of the present invention to be able to provide a method of making body protectors of protective material which give a reasonable degree of protection and which are not harmful should they become damaged.

US-A-4 507 801 describes a protective garment made of stretch material having pockets over the areas to be protected, with pads inserted into the pockets. The pads comprise a rigid centre layer of heat formable material covered with a plurality of layers of closed cell foam material. The centre layer is suitably a polycarbonate or polyethylene plastic; and the foam material is suitably a heat moldable closed cell polyethylene foam plastic.

GB-A-1556357 describes a method of making a semi-rigid protective material for use on a body, which comprises making a laminate of a high density polyethylene foam between a layer of low density foamed plastics material and a layer of a flexible, impact resistant plastics material, and moulding the resulting laminate into shape.

We have now devised a method for making an improved such material, in which method the high density polyethylene foam is in the form of one or more pieces and said lamination process comprises positioning the piece or pieces of high density polyethylene foam between the sheet of flexible polymeric material of high impact strength and the low density foam, heating the entire assembly to between 110°C and 200°C for approximately 2 minutes under a vacuum blanket pressure of 0.2 bar, and then moulding said laminate into shape at a temperature between 80°C and 160°C for 2 minutes with a vacuum blanket pressure of 0.4 bar.

Other layers of plastics material may also be incorporated into the laminate.

The polymer sheet is preferably of thickness in the region of 1.5mm.

The high density polyethylene foam is preferably of thickness in the region 3mm.

The low density foam may be of any thickness between 5 and 15mm, depending on the intended applications of the material.

One or more straps may be attached during the method and are preferably located between the high density polyethylene foam layer and the low density foamed plastics material layer.

Once the laminate is formed in the mould, it will substantially retain the shape of the mould and therefore fit where appropriate around the body of the wearer.

An embodiment of the present invention will now be more particularly described by way of example and with reference to the accompanying drawings, in which:
FIGURE 1 shows schematically a back protector embodying the invention;
FIGURE 2 shows a shin pad embodying the invention; and
FIGURE 3 is a cross-section through a median portion of the shin pad of Figure 2.

Referring now to the drawings, and in particular Figure 3, there is shown a cross-section of material made according to the method of the invention. An outer layer 1 comprises a film of low density polyethylene, high density polyethylene or polypropylene, generally of thickness in the region of 1.5 mm. Such materials are sold under the trade names Courthene (Registered Trade Mark), Hilex (Registered Trade Mark) and Propylex (Registered Trade Mark).

An inner layer 2 is formed of a crosslinked closed cell low density polyethylene or EVA foam. Suitable materials are sold under the trade name Plastazote (Registered Trade Mark) and Evazote (Registered Trade Mark). This inner layer 2 may vary in thickness depending on the function the protector is to perform. For example, in the case of the shin pads it is only 5 mm thick and for the back protector it may be 10 mm thick. In fact, in some cases it nay be as much as 15 mm thick.

Between the inner and outer layers is a central layer 3 of high density polyethylene foam, generally of thickness in the region of 3 mm. The preferred material for this layer is an irradiation crosslinked polyethylene foam sold under the trade name Alveolit (Registered Trade Mark). This central layer 3 is present only over those areas which need most protection, for example over the shin and ankle bones in the shin guard or over the spine and kidneys in the back protector.

The material is made by a process of lamination in a vacuum mould. The piece or pieces of high density polyethylene foam are placed onto the layer of plastics film in position as required and the low density foam is placed on top.

The assembly is then placed on a flat platen and heated to 110 - 200°C depending on the material of the sheet. For polypropylene, 200° is more appropriate or for polyethylene, lower temperatures are needed. The laminate is formed after two minutes at a vacuum blanket pressure of 0.2 bar when the sheet becomes welded to the low density foam around its edges.

The laminate so formed may then be moulded into the required shape in an epoxy vacuum mould preferably operating at a vacuum blanket pressure of 0.4 bar. The moulding time is 2 minutes and the temperature 90°C.

The laminate may incorporate other layers. For example, a laminate may incorporate a layer of polycarbonate plastics material, such as is sold under the trade names RIAG or LEXAN. This layer is disposed between the inner and outer layers, adjacent to one or other of them. Such a laminate may be effective as body armour, at least against stabbing with a knife or other pointed implement. In such cases, the layer of polycarbonate resin may be of a thickness in the region of 3mm.

Another alternative, or indeed additional layer may be of a very low density closed cell polymer foam. This can give buoyancy properties to the protective material, enabling it to be used as a protective life jacket.

One further layer which may be added is of a medium density open celled polyurethane foam available under the trade name CONFOR. This material is highly absorbent of energy and has a slow rate of recovery after deflection. It can be incorporated within the interior of the laminate and can be shaped to conform with the general outline of the protective article including it, even where the article is quite sharply bent.

## Claims

1. A method of making a semi-rigid protective material for use on a body, which comprises making a laminate (1,2,3) of high density polyethylene foam (3) sandwiched between a layer of low density foamed plastics material (2) and a sheet (1) of flexible polymeric material of high impact strength, and moulding the resulting laminate into shape; characterised in that the high density polyethylene foam (3) is in the form of one or more pieces and in that said lamination process comprises positioning the piece or pieces of high density polyethylene foam (3) between the sheet (1) and the low density foam (2), heating the entire assembly (1,2,3) to between 110°C and 200°C for approximately 2 minutes under a vacuum blanket pressure of 0.2 bar, and then moulding said laminate into shape at a temperature between 80°C and 160°C for 2 minutes with a vacuum blanket pressure of 0.4 bar.

2. A method as claimed in claim 1, wherein the polymer sheet is of thickness in the region of 1.5mm.

3. A method as claimed in either claim 1 or claim 2, wherein the high density polyethylene foam is of thickness in the region of 3mm.

4. A method as claimed in any one of the preceding claims, wherein the low density foam is of a thickness between 5 and 15mm.

5. A method as claimed in any one of the preceding claims, wherein the laminate is moulded to shape at a temperature in the region of 90°C.

6. A method as claimed in any one of claims 1 to 4, wherein a layer of polycarbonate resin is provided and placed on said sheet of high impact strength polymer either before or immediately after the piece or pieces of high density polyethylene foam are placed thereon.

7. A method as claimed in claim 6, wherein the layer of polycarbonate resin has a thickness in the region of 3 mm.

8. A method as claimed in either claim 6 or claim 7, wherein the laminate is moulded to shape at a temperature in the region of 150^{°}C.

9. A method as claimed in any one of the preceding claims, further comprising placing a layer of open cell polyurethane foam at such a stage that it lies between the sheet of high impact strength polymer and the layer of low density foamed plastics material.

10. A method as claimed in any one of the preceding claims, further comprising placing a layer of closed cell foam into the laminate, whereby the produced article has buoyancy properties.

11. A method as claimed in any one of the preceding claims, wherein one or more straps are attached during the method and are located between the high density polyethylene foam layer and the low density foamed plastics material layer.

12. A method according to any of claims 1 to 11, wherein the layer (2) of low density foamed plastics material is of polyethylene or EVA polymer.

13. A method according to any of claims 1 to 12, wherein the sheet (1) of high impact strength flexible polymer is of low or high density polyethylene or polypropylene.

## Patentansprüche

1. Eine Methode zur Herstellung eines halbharten Schutzmaterials zur Verwendung auf einem Körper, das die Herstellung eines Schichtstoffs (1, 2, 3) aus Polyethylenschaum hoher Dichte (3), der zwischen einer Schicht aus geschäumtem Kunststoffmaterial niedriger Dichte (2) und einer Folie (1) aus flexiblem Polymermaterial mit hoher Schlagzähigkeit angeordnet ist, und das Bilden des entstandenen Schichtstoffs zu einer Form umfaßt, und die dadurch gekennzeichnet ist, daß der Polyethylenschaum (3) hoher Dichte in Form von einem oder mehreren Stücken ist und daß der genannte Laminierungsprozeß die Anordnung des Stückes bzw. der Stücke des Polyethylenschaums (3) hoher Dichte zwischen der Folie (1) und dem Schaum (2) niedriger Dichte, die Erhitzung der gesamten Baugruppe (1, 2, 3) auf zwischen 110 °C und 200 °C für die Dauer von etwa zwei Minuten unter einem Gesamtunterdruck von 0,2 bar und anschließendes Bilden des genannten Schichtstoffs zu einer Form bei einer Temperatur zwischen 80 °C und 160 °C für die Dauer von zwei Minuten unter einem Gesamtunterdruck von 0,4 bar umfaßt.

2. Eine Methode laut Anspruch 1, bei der die Polymerfolie eine Dicke im Bereich von 1,5 mm aufweist.

3. Eine Methode laut Anspruch 1 oder Anspruch 2, bei der der Polyethylenschaum hoher Dichte eine Dicke im Bereich von 3 mm aufweist.

4. Eine Methode laut einem der vorgenannten Ansprüche, bei der der Schaum niedriger Dichte eine Dicke zwischen 5 und 15 mm aufweist.

5. Eine Methode laut einem der vorgenannten Ansprüche, bei der der Schichtstoff bei einer Temperatur im Bereich von 90 °C zu einer Form gebildet wird.

6. Eine Methode laut einem der Ansprüche 1 bis 4, bei der eine Schicht aus Polycarbonatharz verwendet und auf besagte Folie aus hochschlagzähem Polymer entweder vor oder unmittelbar nach dem Aufbringen des Stückes bzw. der Stücke aus Polyethylenschaum hoher Dichte aufgebracht wird.

7. Eine Methode laut Anspruch 6, bei der die Schicht aus Polycarbonatharz eine Dicke im Bereich von 3 mm aufweist.

8. Eine Methode laut Anspruch 6 oder Anspruch 7, bei der der Schichtstoff bei einer Temperatur im Bereich von 150 °C zu einer Form gebildet wird.

9. Eine Methode laut einem der vorgenannten Ansprüche, die des weiteren das Aufbringen einer Schicht aus offenzelligem Polyurethanschaum derart umfaßt, daß dieser zwischen der Folie aus hochschlagzähem Polymer und der Schicht aus geschäumtem Kunststoffmaterial niedriger Dichte liegt.

10. Eine Methode laut einem der vorgenannten Ansprüche, die außerdem das Aufbringen einer Schicht geschlossenzelligen Schaums auf den Schichtstoff beinhaltet, wobei der hergestellte Artikel schwimmfähig ist.

11. Eine Methode laut einem der vorgenannten Ansprüche, bei der ein Gurt oder mehrere Gurte während des Verfahrens angebracht werden und zwischen der Schicht aus Polyethylenschaum hoher Dichte und der Schicht aus geschäumtem Kunststoffmaterial niedriger Dichte angeordnet werden.

12. Eine Methode laut einem der Ansprüche 1 bis 11, bei der die Schicht (2) des geschäumten Kunststoffmaterials niedriger Dichte aus Polyethylen oder EVA-Polymer besteht.

13. Eine Methode nach einem der Ansprüche 1 bis 12, bei der die Folie (1) aus hochschlagzähem, flexiblem Polymer aus Polyethylen oder Polypropylen niedriger oder hoher Dichte besteht.

## Revendications

1. Une méthode permettant de fabriquer un matériau protecteur semi-rigide à poser sur le corps, consistant à fabriquer un laminé (1,2,3) de mousse polyéthylène haute densité (3) placée entre une couche de matériau plastique expansé basse densité (2) et une feuille (1) de matériau polymère flexible très résistant aux chocs, et à donner forme au laminé ainsi obtenu par moulage; le processus est le suivant: la mousse polyéthylène haute densité (3) est sous la forme d'une pièce ou plus et ledit procédé de laminage consiste à poser la ou les pièces de mousse polyéthylène haute densité (3) entre la feuille (1) et la mousse basse densité (2), à chauffer l'ensemble (1,2,3) à une température comprise entre 110°C et 200°C pendant environ 2 minutes, à une pression de coussin de moulage sous vide de 0,2 bar, et à donner forme audit laminé par moulage à une température entre 80°C et 160°C pendant 2 minutes, la pression de coussin de moulage sous vide étant de 0,4 bar.

2. Une méthode conforme à la sollicitation 1, selon laquelle la feuille polymère fait environ 1,5mm d'épaisseur.

3. Une méthode conforme à la sollicitation 1 ou 2, selon laquelle la mousse polyéthylène haute densité fait environ 3mm d'épaisseur.

4. Une méthode conforme aux sollicitations précédentes quelles qu'elles soient, selon laquelle la mousse basse densité fait environ 5 à 15mm d'épaisseur.

5. Une méthode conforme aux sollicitations précédentes quelles qu'elles soient, selon laquelle on donne forme au laminé par moulage à une température d'environ 90°C.

6. Une méthode conforme aux sollicitations 1 à 4 quelles qu'elles soient, selon laquelle on place une couche de résine de polycarbonate sur ladite feuille en polymère très résistant aux chocs, soit avant soit immédiatement après que la ou les pièces de mousse polyéthylène haute densité y ai(en)t été posée(s).

7. Une méthode conforme à la sollicitation 6, selon laquelle la couche de résine de polycarbonate fait environ 3mm d'épaisseur.

8. Une méthode conforme à la sollicitation 6 ou 7, selon laquelle on donne forme au laminé par moulage à une température d'environ 150°C.

9. Une méthode conforme aux sollicitations précédentes quelles qu'elles soient, et consistant à ajouter une couche de mousse polyuréthane à alvéoles ouvertes de façon à ce qu'elle soit située entre la feuille de polymère très résistant aux chocs et la couche de matériau plastique expansé basse densité.

10. Une méthode conforme aux sollicitations précédentes quelles qu'elles soient, et consistant à ajouter une couche de mousse à alvéoles fermées dans le laminé, conférant ainsi des propriétés de flottabilité à l'article obtenu.

11. Une méthode conforme aux sollicitations précédentes quelles qu'elles soient, selon laquelle on attache une bande ou plus pendant le processus et on la (les) place entre la couche de mousse polyéthylène haute densité et la couche de matériau plastique expansé basse densité.

12. Une méthode conforme aux sollicitations de 1 à 11 quelles qu'elles soient, selon laquelle la couche (2) de matériau plastique expansé basse densité est constitué de polyéthylène ou de copolymère éthylène.

13. Une méthode conforme aux sollicitations de 1 à 12 quelles qu'elles soient, selon laquelle la feuille (1) de polymère flexible très résistant aux chocs est constituée de polyéthylène haute densité ou de polypropylène.
